

J. H. LANGROCK.

MAKING STENCILS.

APPLICATION FILED JAN. 18, 1913.

1,103,005.

Patented July 7, 1914.



Witnesses.

Shelia Briate  
P. E. Schrell

Inventor:  
Joseph H. Langrock  
By his Attorney  
Geo. F. Munn

# UNITED STATES PATENT OFFICE.

JOSEPH H. LANGROCK, OF NEW YORK, N. Y., ASSIGNOR TO LANGROCK BROS. COMPANY,  
A CORPORATION OF NEW YORK.

## MAKING STENCILS.

1,103,005.

Specification of Letters Patent.

Patented July 7, 1914.

Application filed January 18, 1913. Serial No. 742,972.

*To all whom it may concern:*

Be it known that I, JOSEPH H. LANGROCK, a citizen of the United States, and a resident of the borough of Brooklyn, city of New York, county of Kings, and State of New York, have invented certain new and useful Improvements in the Making of Stencils, of which the following is a specification.

My invention relates to a stencil the base 10 of which is a foraminous fabric, such for instance as that known as organdie or muslin, the interstices in which are filled up more or less, in whole or in part, with an insoluble pigment which represents the negative portion 15 of the design to be reproduced.

The accompanying drawing is a diagrammatic representation of a stencil made in accordance with my invention, the size of the mesh being necessarily increased for 20 clearness of illustration.

In making my stencil I first stretch a base B, of organdie or muslin or other suitable foraminous fabric upon a frame F, which holds the material taut and facilitates manipulation. For convenience I herein designate the face of the stencil fabric as that outside the frame, and the back of the fabric as that within the frame. I then apply to the face of the stencil fabric a layer or 25 coating of pigmentary vehicle P, say for instance a mixture of approximately seventy-five per cent. of zinc oxid, zinc white, or a suitable paint or pigment, with twenty-five per cent. of a suitable varnish drier, al- 30 though I do not limit myself to any particular pigment or filler nor to any particular vehicle, nor to the proportions thereof, the essential feature in this respect being 35 the use of suitable filling material in conjunction with a vehicle which is also what is technically known as a drier. The next 40 step is to scrape off the excess of pigmentary vehicle from the face of the fabric, which operation necessarily forces more or less of 45 the material through the mesh to the back of the fabric. This protrusion of the material through the mesh is scraped off, and the evenly coated stencil base is then subjected to a damp heat until "half dry" or 50 sufficiently so to facilitate the manipulation to follow. A positive or relief design block or plate is used to effect the desired displacement and disposition of the pigmentary filling material within and upon the fabric. 55 This block may consist of a manually en-

graved relief plate, or of one produced by photo-gravure or any other appropriate process or method, the essential feature being that the raised or cameo portions of the block face shall represent the positive lines 60 or surfaces in the print to be obtained from the completed stencil (or in other words the clear portions of the stencil) while the intaglio or depressed portions of the face of the block or plate represent the solid or 65 filled in portions of the mesh of the stencil, and consequently the clear portions of the print to be obtained therefrom. Previous to use the face of this relief block is covered with a zinc or other suitable powder the excess of which is wiped or brushed off, leaving the raised portions of the design free and smooth, but filling the depressed portions of the design with the powder. The face of the half dry stencil fabric is applied 70 to the face of the design block in such manner that the raised or positive portions of the design force the pigmental vehicle through the mesh. The back of the fabric is then scraped by the use of a thin flexible 75 blade, with the result that while the material forced through the mesh by the positive portions of the design is removed, leaving such portions of the mesh free and clear, filling material is also forced back through 80 the portions of the mesh overlying the depressed portions of the design and into contact with the powder therein contained, which powder, or the greater portion thereof, is taken up and assimilated by the pigmental vehicle thus forced through the mesh, and becomes a component part thereof. The stencil fabric after such treatment 85 is removed from the design block and dried, the resulting stencil showing the negative 90 or filled portions of the mesh in slightly raised relief upon the face of the stencil, with the intervening portions of the mesh clear and unobstructed for the passage of the paint or other marking material to represent the positive portions of the print to 95 be obtained from the stencil. This protrusion of the filled or negative portions of the design on the face of the stencil is an advantage in that it spaces the stencil more 100 or less away from the surface to be printed upon so that even the more delicate and intricate portions of the design are insured an adequate quantity or layer of paint, ink or other printing vehicle. Incidentally the use 105 110

of the powder on the design block facilitates the removal of the stencil therefrom, but the more important function of the powder is to unite with the pigmental vehicle forced into the depressed portions of the design as hereinbefore set forth.

Obviously my relief design block or plate may be used in the making of innumerable stencils, so that the initial cost of said block or plate is offset by its permanence, and the 10 ease and cheapness with which stencils may be reproduced or duplicated.

What I claim as my invention and desire to secure by Letters Patent is,

- 15 1. The herein described process of making stencils, which consists in coating a foraminous fabric with a pigmentary vehicle, removing the excess of such vehicle from one side of the fabric and forcing portions 20 thereof through the meshes to the other side of the fabric, removing such forced-through portions, subjecting the stencil base to a damp heat, and applying the face of the fabric to a relief design surface and forcing by 25 the raised portions thereof the pigmentary vehicle through the mesh of the fabric to the other side thereof and finally removing the excess of such pigmentary vehicle.
- 30 2. The process of making stencils herein set forth, consisting in casing a taut foraminous fabric with a pigmental vehicle,

removing the excess thereof from the face and back of the fabric, applying the face of the latter to a relief design block or 35 plate the depressed portions of which contain a powder adapted to assimilate with the pigmental vehicle, applying pressure in such manner that the raised portions of the design force the pigmental vehicle through 40 the mesh to the back thereof, removing the excess of pigmental material from the back and forcing a portion of it through the mesh and into the depressed portions of the design surface, whereby a relief stencil 45 is formed substantially as herein set forth.

3. The herein described process of making stencils, which consists in coating a foraminous fabric with a pigmentary vehicle, removing the excess of such vehicle from one side of the fabric and forcing portions 50 thereof through the meshes to the other side of the fabric, removing such forced-through portions, and applying the face of the fabric to a relief design surface and forcing by 55 the raised portions thereof the pigmentary vehicle through the mesh of the fabric to the other side thereof and finally removing the excess of such pigmentary vehicle.

JOSEPH H. LANGROCK.

Witnesses:

GEO. WM. MIATT,  
LILLIA MIATT.